# EUROPEAN PATENT SPECIFICATION

(11) **EP 0 177 328 B1**
(45) Date of publication and mention of the grant of the patent: **04.04.1990**
(21) Application number: 85306999.5
(22) Date of filing: 01.10.1985
(51) Int. Cl.: G03C 1/498

(54) **Photothermograhic accelerators for leuco diazine, oxazine, and thiazine dyes**
Photothermographische Beschleuniger für Leuco-diazin, -oxazin- und thiazinfarbstoffe
Accélérateurs photothermographiques pour leuco-colorants diaziniques, oxaziniques et thiaziniques

(30) Priority: 01.10.1984 US 656690
(43) Date of publication of application: 09.04.1986
(73) Proprietor: MINNESOTA MINING AND MANUFACTURING COMPANY, St. Paul, Minnesota 55133-3427 (US)
(72) Inventor: Bellus, Peter A. Minnesota Mining and, P.O. Box 33427 St. Paul Minnesota 55133 (US); Frenchik, Robert A. Minnesota Mining and, P.O. Box 33427 St. Paul Minnesota 55133 (US)
(74) Representative: Baillie, Iain Cameron

(56) References cited:
- EP-A- 0 061 898
- DE-A- 2 446 892
- US-A- 4 452 883

## Description

### Field of the Invention

The present invention relates to photothermographic color constructions. The invention also relates to two- or three-color separation photothermographic recording systems utilizing such constructions.

### Background Art

Photothermographic imaging systems are those imaging materials which, upon first being exposed to light in an imagewise fashion, produce an image when subsequently heated. The exposure to light or other radiation photoactivates or photodeactivates a component in the imageable element and subsequent heating causes an image forming reaction to differentially occur in exposed and unexposed regions.

Silver halide photothermographic imaging materials, often referred to as "dry silver" compositions because no liquid development is necessary to produce the final image, have been known in the art for many years. These imaging materials basically comprise a light-insensitive, reducible silver source, a light-sensitive material which generates silver when irradiated, and a reducing agent for silver ion in the silver source. The light-sensitive material is generally photographic silver halide which must be in catalytic proximity to the light-insensitive silver source. Catalytic proximity is an intimate physical association of these two materials which enables catalysis of the reduction of the silver source by silver specks formed on the silver halide. Exposure of the silver halide to light produces small clusters of silver atoms. The imagewise distribution of these clusters is known in the art as the latent image. This latent image generally is not visible by ordinary means and the light-sensitive article must be further processed in order to produce a visual image. The visual image is produced by the catalytic reduction of silver ions which, as already noted, are in catalytic proximity to the specks of the latent image.

The silver source used in this area of technology is a material which contains a reducible source of silver ions. The earliest and still preferred source comprises silver salts of long chain carboxylic acids, usually of from 10 to 30 carbon atoms. The silver salt of behenic acid or mixtures of acids of like molecular weight have been primarily used. Salts of other organic acids or other organic materials such as silver imidazolates have been proposed, and U.S. Patent No. 4,260,677 discloses the use of complexes of inorganic or organic silver salts as image source materials.

Color-forming, "dry silver" imaging systems are known in the photographic art. Color-formation is based on the oxidation/reduction reaction between the light-exposed silver salt of a fatty acid which has been halidized and dye-sensitized to a specific wavelength and is used with a chromogenic developer in the presence of elevated temperature. For example, U.S. Patent No. 3,531,286 teaches the inclusion of color coupler components such as a p-phenylenediamine developer and a phenolic or active methylene coupler in close proximity to the light-sensitive emulsion. J. W. Carpenter and P. W. Lauf, Research Disclosure No. 17029, issued June 1978, review prior art relating to photothermographic silver halide systems which include color formation.

US Patent No. 4,021,240 discloses the use of sulfonamidophenol reducing agents and four equivalent photographic color couplers in thermographic and photothermographic emulsions to produce dye images including multicolor images.

US Patent No. 3,985,565 discloses the use of certain class of phenolic type photographic color couplers in photothermographic emulsions to provide a color image.

US Patent No. 4,021,250 (equivalent to DE-A-2,446,392) discloses the use of 0.0025 percent leuco thiazine dye as a shelf life extender in a photothermographic system for generating a black and white image, the system comprising an organic silver salt, a catalytic amount of a photosensitive silver halide, a reducing agent, and a binder. One example discloses 1.87 percent chlorothymol and 0.126 percent phthalazinone as the image producing reactants. The leuco thiazine dye can be used in combination with other acid stabilizers.

Leuco methylene blue, a thiazine dye, is known to be useful in recording systems. US Patent No. 2,646,367 discloses a carbonless copy system using, for example, benzoyl leuco methylene blue as the color forming agent. US Patent No. 3,447,944 discloses a thermographic copy system utilizing leuco methylene blue and its derivatives as color former. US Patent No. 4,309,255 relates to leuco methylene blue in electrochromic recording paper.

Japanese laid-open patent document 59-5239 discloses a 2-sheet, positive-acting, light-sensitive, heat-developable, diffusion, image transfer construction.

### Summary of the Invention

The present invention comprises a single-sheet, negative-acting photothermographic construction comprising at least one light-sensitive, color-forming element on a support base, the element comprising a light-sensitive and non light-sensitive silver source, a binder, an oxidizable leuco phenazine, phenoxazine, or phenothiazine dye as the sole reducing agent for said silver sources, and as development accelerator a carboxylic acid, Lewis acid or Bronsted acid, wherein the image color is provided by the oxidized form of said leuco dye. Any oxidizable leuco phenazine, phenoxazine, or phenothiazine dye known in the art is useful in the present invention.

The light-sensitive element may optionally include a silver halide. The oxidized forms can have colors ranging from turquoise to yellow.

The photothermographic portion of the element can be any imageable layer or layers which are photosensitive and developable by being heated (e.g., on a heated drum roll or by exposure to infrared radiation), preferably in the temperature range of approximately 65 to 180°C (150 to 350°F). Particularly important are silver halide photothermographic systems comprising silver halide, a silver source material in catalytic proximity to the silver halide, and a reducing agent for silver ion in a binder, these systems being commonly known as "dry silver" construction. These systems may be in a single layer or in a plurality of layers as is well known in the art.

The color-forming element of the present invention can be useful in a two or three color separation photothermographic recording system. In such a system it may be required to provide in a topcoat layer a "barrier polymer" which is impervious to an upper adjacent color layer. Such constructions are described, for example, in U.S. Patent Nos. 4,460,681 and 4,452,883.

In the present application:
"leuco dye" means a colorless or slightly colored dye which can be oxidized to a colored form;
"aryl" means phenyl or naphthyl;
"arylene" means phenylene or naphthylene;
"lower alkyl" means alkyl containing 1 to 4 carbon atoms;
"lower alkoxy" means alkoxy containing 1 to 4 carbon atoms;
"aliphatic" means a straight-chain or branched-chain hydrocarbon;
"halogen" means fluorine, chlorine, bromine or iodine; and

"in association with" means in the same layer or in a layer contiguous thereto. For example, the location of the photosensitive silver halide in the photothermographic element or composition of the invention is such that will enable catalytic action. The described photosensitive silver halide can accordingly be in the same layer as or in a layer contiguous to the described oxidation-reduction image- forming combination (i.e., the silver salt oxidizing agent such as silver behenate or silver stearate and the reducing agent and development modifier of the present invention).

### Detailed Description

A preferred embodiment of the present invention comprises a single-sheet, negative-acting, photothermographic element on a support base, said element comprising a silver source, optionally silver halide, a leuco dye as the sole reducing agent for silver ion, a binder, and a development accelerator, wherein
a) said leuco dye comprises a phenazine, phenothiazine, or phenoxazine leuco dye having the formula wherein
   X can be -S-, -0-, or -NQ-;
   each R can be the same or different and is independently selected from
      1) hydrogen,
      2) an unsubstituted aryl or alkyl group or these groups substituted by up to four groups selected from alkyl, alkoxy, cyano, hydroxy, halogen, nitro, mercapto, alkylsulfonyl, arysulfonyl, and Z, where Z is as defined below, wherein all alkyl and alkoxy groups have 1 to 20 carbon atoms, and preferably are lower alkyl and alkoxy, and
      3) Z, wherein Z can be wherein each Q can be the same or different and is independently selected from
         1) hydrogen,
         2) an unsubstituted aryl or alkyl group or these groups substituted by up to four groups selected from alkyl, alkoxy, cyano, hydroxy, halogen, nitro, mercapto, alkylsulfonyl, arysulfonyl, and Z, where Z is as defined above, wherein all alkyl and alkoxy groups have 1 to 20 carbon atoms, and preferably are lower alkyl and alkoxy; and
   R' is the same or different and can be independently selected from hydrogen, halogen, alkyl or alkoxy of 1 to 6 carbon atoms or by these groups substituted by up to 3 halogen atoms; and
   L can be Z or hydrogen; with the proviso that R and L can have up to a total of 5 carbonyl and sulfonyl groups, preferably up to 3 carbonyl and sulfonyl groups; and
b) said development accelerator comprises at least one acid selected from:
   1) a carboxylic acid having the formula wherein
      n is an integer having the value 1 to 4, preferably 1 to 3,
      R¹⁰ is a group which is unsubstituted or substituted by at least one group selected from amino, hydroxyl, aryl, C₁ to C₄ alkyl, C₁ to C₄ alkoxy, cyano sulfonyl, mercapto, nitro, halogen, and Z, wherein Z is as defined above, wherein
      when n is 1,
      R¹⁰ is selected from the group consisting of alkyl, alkenyl, aryl, and phenylalkyl, all having up to 10 carbon atoms, and
      when n is 2, 3, or 4,
      R¹⁰ is selected from the group consisting of alkenylene, alkylene, and arylene, all having up to 14 carbon atoms;
   2) a Lewis acid salt selected from halide, nitrate, sulfate, sulfonate, and carboxylate salts such as ammonium and alkyl-substituted ammonium nitrates, nitrates of Ni, Zn, Al, Cu, and Hg, and chloride of mercury II; and
   3) Bronsted acid selected from sulfonic and sulfinic acids, phenols, phosphonic and phosphinic acids, and sulfimides.

The above-defined leuco dyes, for example, can have a molecular weight up to 2000, preferably up to 700, and the carboxylic acids can have a molecular weight up to 500, preferably up to 400.

The preferred photothermographic construction of the present invention is of the "dry silver" type. The color-forming element which can provide an image ranging from cyan to yellow, including, magenta, red, violet, purple or blue can be of unitary construction or the light-sensitive layer may be in association with the leuco dye, i.e., in a bilayer construction. Single layer constructions must contain the silver source material, the silver halide, the developer, and the development accelerator in the same layer. In a bilayer construction the light-sensitive layer has a topcoat layer which comprises the leuco dye and acid material. Dry silver bilayer constructions must contain the silver source and silver halide in one emulsion layer (usually the layer adjacent the substrate). The other ingredients can be in the same layer, a second layer, or both layers. Optional additional materials include toners, coating aids, and other adjuvants.

Photothermographic color constructions of the present invention incorporate at least one spectrally- sensitized color-forming element according to the present invention to produce a single or multi-color photothermographic color recording system. When at least two color-forming elements are present, the spectral sensitization may be to a pair of colors such as two of black, yellow, red, green, blue, and purple provided that each color-forming element is sensitized to a portion of the spectrum at least 60 nm different from the other color-forming element(s), and each color-forming layer forms a visible dye having a maximum absorbance at least 60 nm different from that of the dye formed in the other color-forming element(s). Preferred pairs of colors to which the construction may be sensitized are yellow-cyan, yellowmagenta, and cyan-magenta. Preferably, a barrier polymer which is impervious to the solvent system of a color construction above it is coated between each pair of color-forming layers. Such a barrier polymer or barrier polymers are essential for the production of good color separation. The test for determining if a barrier polymer is impermeable to the solvent of the next layer can be simply performed. Such a test is described in U.S. Patent No. 4,452,883. The photothermographic color construction may comprise three different monocolor-forming layers to provide a 3-color forming system.

The oxazine and thiazine leuco dyes and dyes of the invention can be prepared as is known in the art by acylation of an unsubstituted phenoxazine or phenothiazine compound to provide an N-acylated phenoxazine or phenothiazine compound. Nitration, in acetic acid, as is known in the art provides, after recrystallization, the 3,7-dinitro phenoxazine or phenothiazine compound. Hydrogenation catalyzed by platinum metal gives the corresponding diamino compounds. Treatment of the diamino compound with the appropriate alkylating or acylating reagent at room temperature in the presence of a base such as pyridine, triethylamine, or sodium hydroxide, gives the diamino substituted leuco dye. To prepare leuco phenazine dyes useful in the present invention a phenylene diamine compound, e.g., N,N-dimethyl p-phenylenediamine and an aniline compound, e.g., N,N-dimethylaniline are combined in a solvent, preferably water, in a reaction vessel and stirred, preferably at room temperature. It is preferred that the reaction be conducted in an aqueous acidic environment. A second aniline compound, e.g., 4-methylaniline is then added to the mixture. The resulting mixture is then stirred and heated for a sufficient period of time to bring about formation of the dye product in free form. To the solution is added an ionizable halide salt, e.g., KI, NaCI, to precipitate the dye product. The solution is then cooled, and the dye collected by filtration and dried in air. Reduction in water in the presence of a water-soluble reducing agent, e.g., sodium dithionite, provides a hydrogen leuco dye. Extraction in a non-reactive water-insoluble solvent (e.g., methylene dichloride) and treatment of the organic portion with a reactive halide compound (e.g., benzoyl chloride) gives the leuco dye.

In a preferred embodiment wherein the photothermographic construction is of the dry silver type, the silver source material, as mentioned above, may be any material which contains a reducible source of silver ions. Silver salts of organic acids, particularly long chain (10 to 30, preferably 15 to 28, carbon atoms) fatty carboxylic acids are preferred. Complexes of organic or inorganic silver salts wherein the ligand has a gross stability constant for silver ion of between 4.0 and 10.0 are also desirable. The silver source material should constitute from about 5 to 70 and preferably from 7 to 30 percent by weight of the imaging layer. The second layer in a two-layer construction would not affect the percentage of the silver source material desired in the single imaging layer.

The silver halide may be any photosensitive silver halide such as silver bromide, silver iodide, silver chloride, silver bromoiodide, silver chlorobromoiodide, silver chlorobromide, etc., and may be added to the emulsion layer in any fashion which places it in catalytic proximity to the silver source. The silver halide is generally present as 0.75 to 15 percent by weight of the imaging layer, although larger amounts up to 20 or 25 percent are useful. It is preferred to use from 1 to 10 percent by weight silver halide in the imaging layer and most preferred to use from 1.5 to 7.0 percent.

Where the construction has more than one color-forming element, the dyes formed from the leuco dyes in the various color-forming layers should of course be different. A difference of at least 60 nm in reflective or transmissive maximum absorbance is required. Preferably the absorbance maximum of dyes formed will differ at least 80 or 100 nm. When three dyes are to be formed, two should differ by at least these minimums, and the third should differ from at least one of the other dyes by at least 150 nm and preferably at least 200 or even at least 250 nm. This will provide a good, full color range for the final image.

In the present invention, the sole reducing agent (developer) for silver ion is the leuco phenazine, phenoxazine, or phenothiazine dye defined above which will reduce silver ion to metallic silver and produce a colored dye. Many representative examples of these dyes are given below in TABLES I and II. The reducing agent should be present as 0.1 to 10 percent by weight of the imaging layer. In a two-layer construction, if the reducing agent is in the second layer, slightly higher proportions, of from about 2 to 15 percent, tend to be more desirable.

Toners such as phthalazinone and phthalazine and others known in the art are not essential to the construction, but may be desirable. These materials may be present, for example, in amounts of from 0.001 to 1 percent by weight.

The binder for the silver coating is selected from well-known natural and synthetic resins such as gelatin, polyvinyl acetals, polyvinyl chloride, polyvinyl acetate, cellulose acetate, ethyl cellulose, polyolefins, polyesters, polystyrene, polyacrylonitrile, polycarbonates, methacrylate copolymers, maleic anhydride ester copolymers, and butadiene-styrene copolymers, for example. When simultaneous coating of layers is used, the binder is selected to coordinate with the solvent used. Copolymers and terpolymers which include the above-stated binders are of course included in these definitions. The preferred photothermographic silver containing binder is polyvinyl butyral. The binders are generally used in a range of from 20 to 75 percent by weight of each layer, and preferably about 30 to 55 percent by weight.

Development modifiers which can be useful in the present invention have been defined above. The acid chosen for a particular light-sensitive element depends on the activity of the leuco diazine, oxazine, or thiazine dye, i.e., upon its tendency to become oxidized to a colored form. More reactive leuco dyes require less acidic materials than to less readily oxidized leuco dyes. For example, Pergascript Turquoise" (a more reactive leuco dye) requires phthalic acid whereas Copikem WM (a less reactive leuco dye) requires a more reactive acid such as 4-nitrophthalic acid. Representative and preferred development modifiers include aromatic carboxylic acids and their anhydrides such as phthalic acid, benzoic acid, chlorinated and nitro- substituted benzoic acids, 1,2,4-benzenetricarboxylic acid, 2,3-naphthalene dicarboxylic acid, tetrachlorophthalic acid, 4-methyl phthalic acid, homophthalic acid, 4-nitrophthalic acid, o-phenylacetic acid, naphthoic acid, naphthalic acid, phthalic anhydride, naphthalic anhydride, tetrachlorophthalic anhydride, 3-nitrophthalic acid; aliphatic carboxylic acids such as malic acid, chloracetic acid, itaconic acid, tartaric acid, benzoylformic acid, and thiodiacetic acid; Bronsted acids, e.g., sulfonic acids such as p-toluene sulfonic acid, phosphonic and phosphinic acids, phenols such as 2,4-dinitrophenol, 2,6-dinitrophenoi, and pentachlorophenol, and other acidic materials such as sulfimides (e.g., saccharin); or Lewis acids including nitrate salts such as nickel nitrate, copper nitrate, mercury nitrate, zinc nitrate, aluminum nitrate, or ammonium nitrate.

Sensitizing dyes useful in the present invention include many compounds known in the art, as well as 454 (prepared as in US Patent No. 2,493,748)

### Ervthrosin (Aldrich Chemical Co., Milwaukee, WI)

### 563 (prepared as in US Patent No. 3,719,495)

### 421 (prepared as in US Patent No. 3,719,495)

The support base or substrate is a transparent or opaque polymeric film. Preferably it is made of such materials as polyester [e.g., poly(ethyleneterephthalate)], cellulose ester (e.g., cellulose acetate, cellulose acetate butyrate, cellulose acetate propionate), polyolefins, polyvinyl resins, and the like.

The coatings can either be made as single layers, as for example by knife-coating or extruding, and dried before the next layer is applied or each monocolor can be dual coated, as for example by dual slide- coating or dual extrusion, i.e., each of the sensitized silver layers with its respective topcoat, which may contain a barrier resin, can be coated together to reduce the number of passes through the coater.

Representative examples of useful leuco diazine, oxazine, and thiazine dyes are given in TABLES I and II below with the Dmin and Dmax values for the bilayer element which was prepared as follows:

Mixing was continued until the Butvar dissolved. Then 1 ml of a solution of 4.3 g ZnC1₂ dissolved 100 ml ethanol was added and mixing continued for 1 hour. The dispersion was coated at 76 micrometer (3 mil) orifice (wet thickness) on a super calendered 691 B Simpson™ photographic paper (Simpson Paper Co., Vicksburg, MI) using a knife coater. The coating was dried 4 minutes at 85°C (185°F).

The five components were mixed until dissolution occurred. To individual samples (8 g) of the topcoat solution 0.05 g of each of the leuco dyes listed in TABLES I and II below were added with mixing. All coatings were at 76 micrometer (3 mil) wet thickness using a Bird applicator over individual samples of the above-described dried silver coating. The construction was dried either at 15 min. at room temperature (21°C), designated condition A, or 3 min at 85°C (185°F), designated condition B. The construction was exposed 20 s to approximately 40904 Ix (3800 fc) using a 3M Model 636 tungsten lamp and then developed at 124°C (255°F) for the specified time on a heated blanket processor.

Objects and advantages of this invention are further illustrated by the following examples, but the particular materials and amounts thereof recited in these examples, as well as other conditions and details, should not be construed to unduly limit this invention.

In the examples the dyes used have the structure:
^{*}Leuco Diazine A
(3M)
MAGENTA

### Preparation of Leuco Diazine A

10 a of Heliotrope B dve (Pfaltz and Bauer Chemical Co., Stamford, CT) was dissolved in 250 ml of water under a nitrogen blanket. Sufficient sodium dithionite was added until all of the color was discharged. 200 ml of methylene chloride was added and the solution was stirred vigorously with a mechanical stirrer. 8 g of benzoyl chloride was added and the pH of the aqueous phase was adjusted to 10 while stirring was maintained for 3 hours. At this time the methylene chloride layer was separated, washed with water, diluted with potassium carbonate solution and again with water. The solution was dried over MgS0₄ and the solvent removed under vacuum yielding a crude product. This material was recrystallized from acetone to give the product leuco diazine A.

### Example 1

The leuco oxazine dye, Pergascript Turquoise S-2G, was tested for photothermographic imaging using it in a silver soap system in the absence of a metal halide with a Lewis acid as development accelerator.

The above solution was milled in a 240-ml glass jar half filled with 12.7 mm glass balls.

### Finished Silver Soap Coating Solution 1B

The following materials were mixed together and coated onto a baryta coated paper at 0.1016 mm (4 mils) and air dried.

Topcoat Formulation

The following solution was prepared to evaluate some acid development modifiers. Master solution 1C

Effect of Nickel Nitrate

A 0.5 ml solution of 0.1 g of nickel nitrate dissolved in 5 ml of methanol and 5 ml of n-methylpyrrolidone was added to 5 g of example master solution 1 C (no acid) and also to 5 g of example master solution 1C containing m-nitrobenzoic acid (0.075 g per 12.1 g master solution 1C). These solutions were coated at 0.1016 mm onto silver soap coating 1 B and air dried. The results are shown in TABLE III.

The data of TABLE III show nickel nitrate acts as a development catalyst without the use of an additional carboxylic acid catalyst.

### Example 2

### Silver Soap Dispersion 2A

A halide sensitized silver soap solution was prepared using the example 2A silver soap homogenate as follows:

This was coated at 0.0762 mm onto 0.0508 mm (2 mil) thick titanium oxide filled polyester film and air dried.

### Topcoat Master Solution 2B

A topcoat master solution was made as follows:

Run using Pergascript Turquoise

Then 0.125 grams of Pergascript Turquoise S2G was added to 10 grams of topcoat master solution 2B. The development modifiers were added and the resulting solutions were coated at 0.1524 mm (6 mils) onto silver soap coating 2A and air-dried. The resulting coated material was then exposed to UV light and developed at 124°C. The results are shown in TABLE IV below.

Run using Copikem-II and Leuco Diazine A

Using the same procedure runs using Copikem-II or Leuco Diazine A in place of the Pergascript Turquoise-S2G were made. The results are shown in TABLE V below.

The data of TABLES IV and V demonstrate the usefulness of various acids as development accelerators with oxazine, thiazine, and diazine leuco dyes in a silver halide-containing photothermographic system.

### Example 3

### Silver Behenate Premix 3A

A silver behenate half soap dispersion was prepared by dispersing 300 grams in 2696 ml of ethanol and 347 ml of toluene by rapid mixing. This dispersion was then homogenized on a Manton-Gaulin Model 15M 8TBA SND homogenizer (Manton-Gaulin CO.) using two passes at 550 kg/cm² (8000 psi) and 225 kg/cm² (4000 psi). Then 389.8 grams of this material were diluted with 113 ml of ethanol. Mixing in 34.7 grams of polyvinyl butyral polymer (Butvar-B76) for 1 hour finished this premix.

### Pergascript Turquoise-S2G Plus Acid in Silver Soap Coating 3B

Evaluation was made of the effect of acid on the oxidation-reduction reaction between Pergascript Turquoise and silver behenate half soap. The following formulation was used for this evaluation.

These solutions were coated at 0.1016 mm onto 0.0508 mm thick titanium oxide filled polyester (3M) and air dried 3 minutes plus 3 minutes 82°C (180°F). Then exposed for 120 seconds to the "Violite" (Allied Litho Supply Co., San Francisco, CA) UV light source (General Electric 15 watt blacklight) through a continuous step tablet. Then processed at 127°C (260°F) on a 3M Model 70 heat blanket processor for 1 to 120 seconds. The densities were measured on a Macbeth densitometer using a red filter. The acids tested are listed in following TABLE VI below.

The 4-nitrophthalic acid was re-evaluated with the addition of 0.4 ml of 0.57 g of mercuric chloride per 100 ml of ethanol and the same repeated with the addition of 3.0 ml of 5 g of tonox™ (R) 201 antioxidant (Shell Chemical Company) to the test solution formulation. These solutions were coated and tested in the same manner as previous samples. The results are listed in TABLE VII below.

The data of TABLE VII show that mercuric chloride can be used as a Lewis acid type development accelerator and as an antifoggant in the present invention with or without an antioxidant.

### Copikem-II Plus Acid In Silver Behenate Coating

Evaluation of the effect of different acids on the oxidation-reduction reaction between Copikem-II and silver behenate half soap was made. The following formulation was used for this evaluation:

These solutions were coated, dried, and processed as described in Example 3B. The acids are listed in TABLE VIII below.

### Leuco Diazine A Plus Acids and Toners in Silver Behenate Coating

Evaluation was made of the effect of acid on the oxidation-reduction reaction using Leuco Diazine A and silver behenate half soap. The following formulation was used for this evaluation:

### Leuco Diazine A Plus Acid and Toners in Silver Behenate Coating

These solutions were coated, dried, and processed as described in 3B. The materials evaluated are listed in TABLE IX below. Measurements were made using a green filter.

The data of TABLE IX shows that a combination of phthazinone plus phthalic acid gave a higher image density than phthalic acid alone.

### Example 4

### Metal nitrate evaluation with leuco oxazine dye

### Silver Behenate Premix 4A

A silver behenate premix was prepared to use in evaluating use of metal nitrate with oxazine and thiazine leuco dyes in a dye sensitized, silver halide containing silver behenate half soap system. The silver behenate homogenate 3A was used.

Sensitized Silver Behenate Premix 4B and 4C

The solution premix 4A was halidized and dye sensitized to green light using the following formula:

This solution was coated at 0.0508 mm onto 0.0508 mm thick titanium oxide filled polyester (3M) and dried for 3 minutes at 77°C (170°F). This was used to evaluate the metal nitrates used in a topcoat containing the leuco dye, phthalic acid, and a polymer.

### Topcoat Master Solution 4D

A topcoat master solution containing Pergascript Turquoise for Lewis acid (nitrate) evaluation was prepared using the following:

Topcoat Solution 4E

The nitrate salts were predissolved in methanol at a concentration of 1 gram per 100 ml. These were added to topcoat master solution 4D to give an equivalent concentration of 2.34 x 10-⁵ moles of metal nitrate per 30 grams of solution. The nitrates which were evaluated are shown in TABLE X with the amounts used in milligrams.

These topcoat solutions were individually coated on top of silver behenate coatings 4B and 4C at an orifice setting of 0.1016 mm and dried for 5 minutes at 77°C (170°F). They were exposed for 10-³ seconds to Xenon flash (EG&G sensitometer) through a continuous tone wedge, then heat developed for 20 seconds at 124°C (255°F) on 3M Model 70 Heat Blanket Processor. The resulting wedges were measured on a computer densitometer using a red filter. The results are shown in TABLES Xl and XII below.

The data of TABLE XI show that the Lewis acid (nitrate) improved the thermal reactivity of the system resulting in higher image densities, gamma angles, and light sensitivity. The image color of the above systems was blue to cyan.

### Example 5

### Nickel nitrate and nickel bromide evaluation as development accelerator with leuco thiazine dye

### Sensitized Silver Behenate Premix 5A

The solution premix 4A prepared in EXAMPLE 4 was halidized and dye sensitized to green light using the following formulation:

This solution was coated at 0.0508 mm onto 0.508 mm thick titanium oxide filled polyester and dried for 3 minutes at 77°C (170°F).

### Topcoat Master Solution 5B

A topcoat master solution containing Copikem-II for metal nitrate evaluation was prepared using the following formulation:

Nickel Nitrate Evaluation

Nickel nitrate and phthalic acid were individually predissolved in methanol at a concentration of 1 gram per 100 mi. Then 0.5 ml of these solutions were added to individual 22.354 gram portions of topcoat master solution 5B. These topcoat solutions were coated over a sensitized silver behenate coating 5A at an orifice setting of 0.1016 mm and dried for 5 minutes at 77°C (170°F). They were exposed, processed, and tested as in EXAMPLE 4. The results are shown in TABLE XIII below:

The data demonstrate the effectiveness of a nitrate salt as development accelerator.

### Example 6

### Combination of other leuco dyes with leuco oxazine and thiazine dyes

### Topcoat Master Solution 6A

A topcoat master solution containing 4-nitrophthalic acid and leuco crystal violet was made to evaluate the effect of combining the oxazine and thiazine leuco dyes with nickel nitrate. The following formulation was used:

The Pergascript Turquoise, Copikem-II and nickel nitrate were predissolved in solvents then added to 20.12 grams of the example topcoat master solution 4G. The following solutions were prepared:

These solutions were coated at 0.0762 mm onto silver behenate coating 5A and dried for 5 minutes at 77°C (170°F). They were exposed, processed, and tested as in Example 4. The results are shown in TABLE XIV halow

All images were bluish-green in color. The data of TABLE XIV show that the combination of the leuco dyes of the invention in combination with other leuco dyes and nickel nitrate gave useful systems.

### Example 7

### Effect of Phthalazine

The effect of phthalazine was evaluated using the following formulation 7A and 7B:

These solutions were coated 0.1016 mm thick onto Silver Behenate Coating 4C and dried for 5 minutes at 77°C (170°F). They were exposed, processed, and tested as in Example 4. The results are shown in TABLE XV below.

The samples were aged for two hours using 2152 milliphots (2000 foot candles), 27°C (80°F), and 60 percent relative humidity. The changes in Dmin are shown in TABLE XV.

The data of TABLES XV and XIV show that conventional development modifiers used in dry silver are also useful in this system. Although phthalazine reduces the thermal reactivity it improves the print stability.

The use of phthalazine with nickel nitrate and Pergascript Turquoise was evaluated in the following formulation.

These solutions were coated at 0.1016 mm onto Silver Behenate Coating 4C and dried for 5 minutes at 77°C (170°F). They were exposed, processed, and tested as in Example 4D. The results are shown in TABLE XVII below.

The data of TABLE XVII show the increased density and sensitivity of the nickel nitrate/phthalazine containing construction. When compared to phthalazine alone, the addition of nickel nitrate was not detrimental to print stability but did improve sensitometry.

### Example 8

### Acids with Oxazine Dye

Cyan Silver Coating 8A (below) was prepared and coated at 3.6 g/m² (0.32 grams per square foot) onto 0.076 mm thick polyester film MELINEX™ TYPE 329 (ICI) using a laboratory hand knife coater. Various acids were used in the construction with the leuco oxazine dye, Pergascript Turquoise 5-2G.

0.064 mm (2.5 mil) orifice; dried 5 min at 82°C (180°F)

The following formulation was used to evaluate acids in a topcoat over the precoated red sensitive silver coating (8A).

The topcoat was coated at a 0.076 mm orifice and dried for 5 minutes at 82°C (180°F). The material was then exposed for 10-³ seconds to an EG&G xenon flash sensitometer. No filter was used. The samples were processed at 124°C (255°F) on a 3M Model 70 heated blanket processor. The dwell times, Dmin and Dmax, are noted with the acid tested in TABLE XX below.

The data of TABLE XX show the usefulness of various acids as development accelerator with Pergascript Turquoise S―2G in color constructions.

### Example 9

### Cyan Oxazine Leuco Dye Developer in Magenta/Cyan Bipack

A dispersion of a silver behenate half soap was made at 10% by weight in a solvent mixture of 90% toluene and 10% ethanol using two passes with a Manton-Gaulin homogenizer, Model 15M, at 550 kg/cm² and 225 kg/cm² (8000 and 4000 psi). This silver soap dispersion is then prepared for coating by the addition of dilution solvents, halide, polymer and sensitizing dye in a selected sequence of time and mixing.

Stop mixing at 340 minutes. 90 grams of EXAMPLE 1 were dye sensitized with 2.7 ml of a #534 dye (green light sensitizer) solution with a concentration of 0.013 g dye/50 ml methanol. This solution was coated on top of a 0.05 mm (2 mil) thick titanium dioxide filled polyester film (3M) using a 0.076 mm (3 mil) orifice on a laboratory hand knife coater. This coating was dried at 81°C (177°F) for 5 minutes.

### Magenta Topcoat 9B

The following topcoat solution was prepared to coat on top of Magenta Silver Coating 9A.

^{*} 8.15 g of 2,6 dichlorophenol and 15.9 g sodium carbonate were dissolved in 300 ml water; then, 150 ml chloroform were added. A solution of 65.9 g potassium ferricyanide in 300 ml water was added and the solution was stirred for 1 hour. The chloroform layer was separated, washed with 5% aqueous sodium hydroxide, dried with MgS0₄ and stripped to yield a dye. One gram of this dye was dissolved in 200 ml diethylether and 0.58 g of t-butylhydroquinone was added. The mixture was allowed to stand for 3 hours. The ether was extracted with 5% aqueous sodium hydroxide. The aqueous layer was separated and acidified with 10% hydrochloric acid. A precipitate formed. This suspension was extracted with ether. The ether was evaporated giving a tan material, the magenta leuco indoaniline dye.

This solution was coated on top of coating 9A using a 0.076 mm (3 mil) orifice and drying at 81°C (177°F) for 5 minutes.

A different dispersion of a silver behenate half soap was made similar to 9A, except that a solvent mixture of 90% ethanol and 10% toluene was used. This silver soap dispersion was used in preparing a red light sensitive coating for the cyan color system which was to be coated on top of the pre-coated magenta color forming system.

50 grams of Cyan Silver Premix 9C solution were dye sensitized with 1.2 ml of MSD 563 dye (red light sensitizer) solution having a concentration of 0.017 grams/50 ml methanol. This was coated on top of the precoated 9A and 9B layers at an orifice of 0.05 mm (2 mils). The coating was dried at 81°C (177°F) for 5 minutes.

### Cyan Color Topcoat 9D

The following topcoat solution was prepared to coat on top of Cyan Silver premix 9C to finish the magenta/cyan color bipack.

This was coated on top of Cyan Silver Premix 9C at an orifice of 0.1016 mm (4 mils) and dried for 5 minutes at 81°C (177°F). The magenta/cyan bipack was now complete and had the following construction:
Base - 0.05 mm thick (2 mil) Ti0₂ filled polyester
1st layer - green light sensitive silver
2nd layer - magenta color developer and development modifiers in barrier polymer
3rd layer - red light sensitive silver
4th layer - cyan color developer and development modifiers in hard topcoat polymer.

This material was exposed to an EG&G (EG&G, Electrooptics Div., Salem, MA) xenon flash sensitometer using the proper light filtration to generate the mono-magenta and mono-cyan colors. A Wratten Number 58 and a Wratten Number 25 were used. The exposed material was then processed at 124°C (255°F) for 20 seconds.

The sensitometry of the bipack is given in TABLE XVIII below.

The data of TABLE XVIII shows that a good color separation was obtained and demonstrates the utility of a two-color system.

### Example 10

### Example of Cyan Oxazine Leuco Dye Developer in Yellow/Magenta/Cyan Tripack

The following will illustrate a three color separation system employing the cyan oxazine leuco dye, pergascript Turquoise.

### Yellow Silver Coating 10A

This solution was prepared by adding 1.5 ml of a #454 dye (blue sensitizer) solution having a concentration of 0.032 grams per 50 cc of methanol to 40 grams of Magenta Silver Coating 9A. This was coated at a 0.1016 mm (4 mil) orifice using a laboratory hand knife coater onto a 0.0508 mm thick (2 mil) titanium dioxide filled polyester film (3M). The coating was dried for 5 minutes at 81°C (177°F).

Charges B and C were mixed together prior to addition to charge A.

Charges B through F were predissolved in charge A before addition of charge G. This solution was coated on top of precoated Yellow Silver Coating 9A at a 0.076 (3 mil) orifice and dried for 5 minutes at 79°C (175°C).

The magenta color forming systems 9A and 9B described in Example 8 were coated on top of the yellow color forming system described above. The resulting material was exposed and processed using the procedure of Example 9. A Wratten Number 47B (blue light) was used for the yellow color.

The sensitometry of this yellow/magenta bipack is given in TABLE XIX below.

The cyan color forming system utilizing Cyan Silver premix 9C and Cyan Silver Coating 9D was coated on top of the yellow/magenta bipack. The sensitometry for the yellow, magenta, and cyan were obtained by the same methods just described. The results showed a good three color separation for copying in color. The sensitometry for the yellow did not change from the bipack and the magenta and cyan were the same as disclosed in the magenta/cyan bipack.

Various modifications and alterations of this invention will become apparent to those skilled in the art without departing from the scope of this invention, and it should be understood that this invention is not to be unduly limited to the illustrative embodiments set forth herein.

## Claims

1. A single-sheet, negative-acting, photothermographic construction comprising at least one light-sensitive color-forming element on a support base, the element comprising a light-sensitive and a non light-sensitive silver source, a binder, an oxidizable leuco phenazine, phenoxazine, or phenothiazine dye as the sole reducing agent for said silver sources, and as develpment accelerator a carboxylic acid, Lewis acid, or Bronsted acid; wherein the image color is provided by the oxidized form of said leuco dye.

2. The construction according to Claim 1, wherein said light-sensitive silver source is silver halide.

3. The construction according to any preceding claim wherein
a) said leuco dye comprises a phenazine, phenothiazine, or phenoxazine leuco dye having the formula wherein
each R is the same or different and is independently selected from
1) hydrogen,
2) an unsubstituted aryl or alkyl group or these groups substituted by up to four groups selected from alkyl, alkoxy, cyano, hydroxy, halogen, alkylsulfonyl, arylsulfonyl, and Z where Z is as defined below, wherein all alkyl and alkoxy groups have 1 to 20 carbon atoms, and
3) Z, wherein Z is
wherein each Q is the same or different and is independently selected from
1) hydrogen,
2) an unsubstituted aryl or alkyl group or these groups substituted by up to four groups selected from alkyl, alkoxy, cyano, hydroxy, halogen, nitro, mercapto, alkylsulfonyl, arylsulfonyl, and Z where Z is as defined above, and wherein all alkyl and alkoxy groups have 1 to 20 carbon atoms;
R' is the same or different and is independently selected from hydrogen, halogen, alkyl or alkoxy of 1 to 6 carbon atoms or these groups substituted by up to 3 halogen atoms; and
X is ―S― -0-, or -NQ-_{;}
L is hydrogen or Z; with the proviso that R and L can have up to a total of 5 carbonyl and sulfonyl groups; and
b) said development accelator comprising at least one acid selected from
1) a carboxylic acid having the formula
wherein
n is an integer having the value 1 to 4,
R¹⁰ is a group which is ubsubstituted or substituted by at least one group selected from amino, hydroxyl, aryl, C₁ to C₄ alkyl, C₁ to C₄ alkoxy, cyano, sulfonyl, mercapto, nitro, halogen atom, and Z, wherein Z is as defined above, wherein when n is 1,
R¹⁰ is selected from the group consisting of alkyl, alkenyl, aryl, and phenylalkyl, having up to 10 carbon atoms, and when n is 2, 3, or 4,
R¹⁰ is selected from the group consisting of alkenylene, alkylene, and arylene, having up to 14 carbon atoms;
2) A Lewis acid salt selected from halide, nitrate, sulfate, sulfonate, and carboxylate salts; and
3) A Bronsted acid selected from sulfonic and sulfinic acids, phenols, phosphonic and phosphinic acids, and sulfimides, wherein the image color is provided by the oxidized form of said leuco dye.

4. The construction according to any preceeding claim wherein said leuco dye is

5. The construction according to any preceding claim wherein said carboxylic acid is selected from substituted benzoic or naphthoic acid.

6. The construction according to any preceding claim wherein said Lewis acid salt is selected from nitrates of Ni, Zn, Al, Cu, Hg, and NH₄+.

7. The construction according to any preceding claim wherein said color-forming element has a unitary layer construction.

8. The construction according to any preceding claim wherein said color-forming element has a bilayer construction.

9. A 2- or 3-color separation photothermographic recording composite comprising a photothermographic construction as claimed in any preceding claim.

## Patentansprüche

1. Negativwirkendes photothermographisches Einzelblattgebilde mit mindestens einem lichtempfindlichen farbbildenden Element auf einem Träger, wobei das Element eine lichtempfindliche und eine nichtlichtempfindliche Silberquelle, ein Bindemittel, ein oxidierbares Laukophenazin, -phenoxazin oder -phenothiazin als einziges Peduktionsmittel für die Silberquellen und als Entwicklungsbeschleuniger eine Carbonsäure, Leweissäure oder Pronstedsäure enthält und die Bildfarbe durch die oxidierte Form bes Leukofarbstoffes gebildet wird.

2. Gebilde nach Anspruch 1, dadurch gekennzeichnet, daß die lichtempfindliche Silberquelle Silberhalogenid ist.

3. Gebilde nach einem der vorhergehenden Ansprüche, dadurch gekennzeichnet, daß
a) der Leukofarbstoff wenigstens teilweise aus einem Phenazin-, Phenothiazin- oder Phenoxazin-Leukofarbstoff der Formel besteht, in der
jedes R-gleich oder unterschiedlich ist und unabhängig ausgewählt ist aus
1) Wasserstoff
2) einer nichtsubstituierten Aryl- oder Alkylgruppe oder einer derartigen Gruppe, die mit bis zu vier Gruppen substituiert ist, die aus Alkyl, Alkoxy, Cyano, Hydroxy, Halogen, Alkylsulfonyl, Arylsulfonyl und Z ausgewählt sind, wobei Z die nachstehend angegebene Redeutung hat und alle Alkyl- und Alkoxygruppen 1 bis 20 Kohlenstoffatome haben, und
3) Z, wobei Z und Q ueweils gleich oder verschieden ist und unabhängig aus Wasserstoff, einer nichtsubstituierten Aryl- oder Alkylgruppe oder einer derartigen Gruppe, die mit bis zu vier Gruppen substituiert ist, die aus Alkyl, Alkoxy, Cyano, Hydroxy, Halogen, Nitro, Mercapto, Alkylsulfonyl, Arylsulfonyl und Z ausgewählt ist, Z die vorstehend angegebene Bedeutung hat und alle Alkyle- und Alkoxygruppen 1 bis 20 Kohlenstoffatome haben
R' gleich oder verschieden ist und unabhängin ausgewählt ist aus Wasserstoff, Halogen, Alkyl oder Alkoxy mit 1 bis 6 Kohlenstoffatomen oder diesen mit bis zu 3 Halogenatomen substituierten Gruppen,
X die Redeutung -S-, -0- oder -NO- hat;
L Wasserstoff oder Z ist;
wobei R und L bis zu insgesamt 5 Carbonyl- und Sulfonylgruppen haben künnen; und
b) der Entwicklungsbeschleuniger wenigstens teilweise aus mindestens einer Säure besteht, die ausgewählt ist aus
1) einer Carbonsäure der Formel in der
n eine ganze Zahl mit einem Wert von 1 bis 4 ist,
R™ eine Gruppe ist, die nichtsubstituiert oder mit minestens einer Gruppe substituiert ist, die aus Amino, Hydroxyl, Aryl, C,- bis C₄-Alkyl, Cᵢ- bis C₄- Alkoxy, Cyano, Sulfonyl, Mercapto, Nitro, einem Halogenatom und Z ausgewählt ist, wobei Z die vorstehend angegebene Bedeutung hat und wenn n gleich 1 ist
R¹⁰ aus der Gruppe ausgewählt ist, die aus Alkyl, Alkenyl, Aryl und Phenylalkyl besteht und bis zu 10 Kohlenstoffatome hat und
wenn n gleich 2, 3 oder 4 ist
R¹⁰ aus der Gruppe ausgewählt ist, die aus Alkenylen, Alkylen und Arylen besteht und bis zu 14 Kohlenstoffatome hat;
2) einem Salz einer Lewissäure, das aus den Halogenid-, Nitrat-, Sulfat-, Sulfonat- und Carboxylatsalzen ausgewählt ist; und
3) einer Bronstedsäure, die aus den Sulfonsäuren, Sulfinsäuren, Phenolen, Phosphon- und Phosphinsäuren und Sulfimiden ausgewählt ist,
wobei die Bildfarbe von der oxidierten Form des Leukofarbstoffs gebildet wird.

4. Gebilde nach einem der vorhergehenden Ansprüche, dadurch gekennzeichnet, daß der Leukofarbstoff ist.

5. Gebilde nach einem der vorhergehenden Ansprüche, dadurch gekennzeichnet, daß die Carboxylsäure aus der substituierten Benzoesäure oder Naphthoesäure ausgewählt ist.

6. Gebilde nach einem der vorhergehenden Ansprüche, dadurch gekennzeichnet, daß das Salz der Lewissäure aus den Nitraten von Ni, Zn, Al, Cu, Hg und NH₄₊ ausgewählt ist.

7. Gebilde nach einem der vorhergehenden Ansprüche, dadurch gekennzeichnet, daß das farbbildende Element eine einzige Schicht bildet.

8. Gebilde nach einem der vorhergehenden Ansprüche, dadurch gekennzeichnet, daß das farbbildende Element zwei Schichten bildet.

9. Photothermographischer Aufnahme-Verbundkörper für 2 oder 3 Farbauszüge mit einem photothermographischen Gebilde nach einem der vorhergehenden Ansprüche.

## Revendications

1. Structure photothermographique monocouche, à effet négatif, comprenant au moins un élément chromogène photosensible sur un support, ledit élément comprenant une source d'argent photosensible et une source d'argent non-photosensible, un liant, un colorant leucodérivé oxydable de type phénazine, phénoxazine ou phénothiazine servant d'agent réducteur unique desdites sources d'argent et, en tant qu'accélérateur de développement, un acide carboxylique, un acide de Lewis ou un acide de Bronsed, la couleur de l'image étant assurée par la forme oxydée dudit colorant leucodérivé.

2. Structure selon la revendication 1, dans laquelle ladite source d'argent photosensible est un halogénure d'argent.

3. Structure selon l'une quelconque des revendications précédentes, dans laquelle
a) ledit colorant leucodérivé comprend un leucocolorant de type phénazine, phénothiazine ou phénoxa-zine, ayant la formule suivant: dans laquelle
les radicaux R sont identiques ou différents, et chacun d'entre eux, indépendamment de l'autre, est choisi parmi L'ensemble comprenant
1) l'hydrogène,
2) les groupes aryle ou alkyle non-substitués, ou ces groupes substitués par jusqu'à quatre groupes choisis parmi l'ensemble comprenant les radicaux alkyle, alcoxy, cyano, hydroxy, halogéno, alkylsulfonyl, arylsulfonyle, et Z, où Z est tel que défini ci-après, tous les groupes alkyle et alcoxy ayant de 1 à 20 atomes de carbone, et
3) Z, où Z est où les radicaux Q sont identiques ou différents et, indépendamment les uns des autres, sont chacun choisis parmi l'ensemble comprenant
1) l'hydrogène,
2) les groupes aryle ou alkyle non-substitués, ou ces groupes substitués par jusqu'à quatre groupes choisis parmi l'ensemble comprenant les radicaux alkyle, alcoxy, cyano, hydroxy, halogéno, mercapto, alkylsulfonyle, arylsulfonyle, et Z, où Z est tel que défini ci-dessus, tous les groupes alkyle et alcoxy ayant de 1 à 20 atomes de carbone;
les radicaux R' sont identiques ou différents et, indépendamment les uns des autres, sont chacun choisis parmi l'ensemble comprenant l'hydrogène, les halogènes, les radicaux alkyle ou alcoxy ayant de 1 à 6 atomes de carbone, ou ces groupes substitués par jusqu'à 3 atomes d'halogène;
X est -S-, -0- ou ―NQ―; et
L est l'hydrogène ou Z;
avec la condition que R et L puissent porter en tout jusqu'à 5 groupes carbonyle et sulfonyle; et
b) ledit accélérateur de développement comprenant au moins un acide choisi parmi:
1) les acides carboxyliques ayant la formule suivante dans laquelle
n est un entier de 1 à 4,
R¹⁰ est un groupe qui est non-substitué, ou substitué par au moins un groupe choisi parmi l'ensemble comprenant les radicaux hydroxyle, aryle, alkyle en C, à C₄, alcoxy en C, à C₄, cyano, suylfonyl, mercapto, nitro, les atomes d'halogène, et Z, où Z est tel que défini ci-dessus, où
quand n vaut 1,
R'^{o} est choisi parmi l'ensemble comprenant les radicaux alkyle, alcényle, aryle et phénylalkyle, ayant jusqu'à 10 atomes de carbone, et
quand n vaut 2, 3 ou 4,
R¹⁰ est choisi parmi l'ensemble comprenant les radicaux alcénylène, alkylène et arylène ayant jusqu'à 14 atomes de carbone;
2) les sels d'acides de Lewis choisis parmi l'ensemble comprenant les halogénures, nitrates, sulfates, sulfonates et carboxylates; et
3) les acides des Bronsted choisis parmi l'ensemble comprenant les acides sulfoniques et sulfiniques, les phénols, les acides phosphoniques et phoshiniques, et les sulfimides,
où la couleur de l'image est assurée par la forme oxydée dudit colorant leucodérivé.

4. Structure selon l'une quelconque des revendications précédentes, dans laquelle ledit colorant leucodérivé est

5. Structure selon l'une quelconque des revendications précédentes, dans laquelle ledit acide carboxylique est choisi parmi l'ensemble comprenant l'acide benzoïque ou l'acide naphtoïque substitués.

6. Structure selon l'une quelconque des revendications précédentes, dans laquelle ledit sel de l'acide de Lewis est choisi parmi les nitrates de Ni, Zn, AI, Cu, Hg et NH₄^{+.}

7. Structure selon l'une quelconque des revendications précédentes, dans laquelle ledit élément chromogène présente une structure monocouche.

8. Structure selon l'une quelconque des revendications précédentes, dans laquelle ledit élément chromogène a une structure bicouche.

9. Composite d'enregistrement photothermographique par séparation à deux ou trois couleurs, comprenant une structure photothermographique selon l'une quelconque des revendications précédentes.
